

# United States Patent Office

3,201,230  
Patented Aug. 17, 1965

1

3,201,230

## AUSTENITIC STAINLESS STEEL

Joseph R. Mitchell, Chicago, and Mary E. Potter, Thornton Township, Cook County, Ill., assignors to United States Steel Corporation, a corporation of New Jersey  
No Drawing. Filed Mar. 16, 1964, Ser. No. 352,314  
5 Claims. (Cl. 75—124)

This application is a continuation-in-part of application Serial No. 117,263, filed June 15, 1961, now abandoned, which was a continuation-in-part of application Serial No. 822,211, filed June 23, 1959, also abandoned.

This invention relates to an aluminum-bearing, non-age-hardening austenitic steel.

Steels possessing a high strength, along with good corrosion resistance and high oxidation resistance are desirable for many missile and aeroplane applications. For such uses, it is essential that the steel be readily hot and cold formable and have good tensile and impact ductile properties. Aluminum is known to provide good scaling properties at high temperatures but prior art steels containing sufficient aluminum to provide enhanced resistance to corrosion or scaling at high temperatures are ferritic and have had such poor cold forging and ductile properties that they were not suitable for the foregoing applications.

It is accordingly an object of the present invention to provide an austenitic steel containing high aluminum contents which combines good corrosion resistance and oxidation resistance at high temperature along with high strength, good tensile and impact ductility and good hot and cold forming properties.

It is another object to provide such properties without the use of expensive alloying ingredients.

We have discovered that the foregoing properties can be obtained in a high aluminum steel if the aluminum content is balanced with respect to chromium and which contains carbon and manganese in proportioned amounts to render the steel austenitic. In its broader aspects the steel will contain the following as essential ingredients.

| Percent   |              |
|-----------|--------------|
| Carbon    | .25 to 1.0   |
| Manganese | 14.0 to 35.0 |
| Silicon   | .25 to 1.0   |
| Chromium  | 4.5 to 8.75  |
| Aluminum  | 3.5 to 8.75  |

wherein the carbon, manganese, chromium and aluminum are balanced to provide an austenitic structure and where-

2

in the chromium and aluminum are balanced within the following limits:

Percent chromium=percent aluminum—1.5  
to

Percent chromium=percent aluminum+1.5

with the total of percent chromium plus percent aluminum being less than 17 and with the remainder iron and other elements in amounts which do not adversely affect the properties.

Desirable results can be obtained with the total percent chromium plus percent aluminum less than 17. However, for the best balance of strength tensile and impact ductility and atmospheric corrosion and oxidation resistance, we prefer the total percent chromium plus percent aluminum to fall within the range of about 9 to 16. Thus a preferred range is as follows:

|           | Percent      |
|-----------|--------------|
| Carbon    | .40 to .90   |
| Manganese | 14.0 to 18.0 |
| Silicon   | .35 to .75   |
| Chromium  | 4.5 to 8.50  |
| Aluminum  | 3.75 to 8.50 |

wherein the carbon, manganese, chromium and aluminum are balanced to provide an austenitic structure and with chromium and aluminum balanced within the following limits:

Percent chromium=percent aluminum—1.5  
to

Percent chromium=percent aluminum+1.5

with the total of percent chromium plus percent aluminum being between 9 and 16 and with the remainder iron and other elements in amounts which do not adversely affect the properties.

Some preferred typical examples of steels are as follows:

|                                     | A     | B     | C     |
|-------------------------------------|-------|-------|-------|
| Carbon                              | 0.50  | 0.80  | 0.90  |
| Manganese                           | 15.00 | 16.00 | 17.00 |
| Silicon                             | 0.50  | 0.50  | 0.50  |
| Chromium                            | 5.00  | 7.00  | 8.00  |
| Aluminum                            | 4.00  | 6.00  | 7.00  |
| Percent Chromium + percent Aluminum | 9     | 13    | 15    |

with the balance substantially iron.

The composition of a number of heats of steel illustrative of our invention are given in the following Table I:

TABLE I.—CHEMICAL COMPOSITION  
GROUP I

| Heat<br>Number | Chemical Composition, Weight Percent |       |       |       |      |      |      |    |    |                           |
|----------------|--------------------------------------|-------|-------|-------|------|------|------|----|----|---------------------------|
|                | C                                    | Mn    | P     | S     | Si   | Cr   | Al   | Mo | Ni | Total<br>percent<br>Cr+Al |
| 1L725          | 0.31                                 | 14.65 | 0.012 | 0.019 | 0.65 | 2.38 | 1.00 | —  | —  | 3.38                      |
| 1L715          | 0.45                                 | 15.10 | 0.011 | 0.014 | 0.43 | 3.78 | 2.70 | —  | —  | 6.46                      |
| 1L547          | 0.45                                 | 14.91 | 0.010 | 0.015 | 0.23 | 4.88 | 3.29 | —  | —  | 8.17                      |
| 1L558          | 0.55                                 | 14.49 | 0.005 | 0.010 | 0.28 | 5.18 | 3.36 | —  | —  | 8.54                      |
| 1L573          | 0.49                                 | 15.09 | 0.016 | 0.013 | 0.89 | 5.25 | 4.17 | —  | —  | 9.42                      |
| 1L640          | 0.85                                 | 17.24 | 0.010 | 0.011 | 0.59 | 6.25 | 6.04 | —  | —  | 12.29                     |
| 1L638          | 0.90                                 | 18.30 | 0.010 | 0.016 | 0.46 | 6.86 | 8.55 | —  | —  | 15.41                     |
| 1L724          | 0.90                                 | 14.08 | 0.010 | 0.018 | 0.52 | 7.52 | 8.17 | —  | —  | 15.69                     |

3  
TABLE I—Continued  
GROUP Ia

|            |      |       |       |       |      |      |      |       |       |       |
|------------|------|-------|-------|-------|------|------|------|-------|-------|-------|
| 1L890..... | 0.93 | 14.21 | 0.103 | 0.016 | 0.50 | 7.66 | 6.45 | 1.00  | ----- | 14.11 |
| 1L881..... | 0.71 | 14.10 | 0.009 | 0.014 | 0.63 | 7.34 | 6.95 | ----- | 0.96  | 14.29 |

GROUP II

|             |      |       |       |       |      |      |      |       |       |
|-------------|------|-------|-------|-------|------|------|------|-------|-------|
| 1L1003..... | 0.61 | 25.55 | 0.016 | 0.104 | 0.63 | 6.43 | 5.31 | ----- | 11.74 |
| 1L1002..... | 0.63 | 27.77 | 0.008 | 0.016 | 0.67 | 6.58 | 5.98 | ----- | 12.56 |
| 1L1005..... | 0.68 | 28.15 | 0.016 | 0.012 | 0.65 | 6.59 | 6.24 | ----- | 12.83 |
| 1L1009..... | 0.62 | 32.88 | 0.010 | 0.014 | 0.28 | 7.21 | 5.80 | ----- | 13.11 |
| 1L1004..... | 0.65 | 28.98 | 0.014 | 0.015 | 0.77 | 6.47 | 6.90 | ----- | 13.37 |
| 1L1006..... | 0.65 | 26.91 | 0.016 | 0.016 | 0.68 | 6.63 | 7.12 | ----- | 13.75 |
| 1L1002..... | 0.90 | 31.50 | 0.015 | 0.015 | 0.74 | 5.52 | 8.25 | ----- | 13.77 |
| 1L095.....  | 0.67 | 34.31 | 0.014 | 0.017 | 0.65 | 7.41 | 6.57 | ----- | 13.98 |
| 1L1009..... | 0.70 | 31.99 | 0.014 | 0.016 | 0.66 | 7.62 | 7.09 | ----- | 14.71 |
| 1L1091..... | 0.76 | 32.04 | 0.015 | 0.015 | 0.69 | 7.42 | 7.86 | ----- | 15.28 |

GROUP IIa

|             |      |       |       |      |      |      |      |       |       |
|-------------|------|-------|-------|------|------|------|------|-------|-------|
| 1L1096..... | 0.68 | 27.74 | ----- | 0.50 | 0.21 | 6.77 | 2.80 | ----- | 6.98  |
| 1L1095..... | 0.69 | 28.98 | ----- | 0.68 | 4.20 | 5.68 | 2.60 | ----- | 9.88  |
| 1L1094..... | 0.67 | 29.81 | ----- | 0.80 | 7.40 | 5.53 | 1.80 | ----- | 12.93 |

Group I steels in Table I have a range of percent chromium plus percent aluminum less than 17 with 14 to 18% manganese and showing carbon levels required to develop an austenitic structure. The Group II steels largely have percent plus percent aluminum levels in the range of 11 to 15% with the manganese sufficiently

high to maintain an austenitic structure with the use of lowered carbon contents. Group Ia steels are modified with molybdenum or nickel and Group IIa are steels modified with molybdenum.

30 The tensile and impact properties of the steels of Table I are given in the following Table II:

TABLE II.—TENSILE AND IMPACT PROPERTIES  
IN THE ANNEALED CONDITION

GROUP I

| Heat Number | Total Cr-Al, Percent | Yield Strength (0.2% Offset), p.s.i. | Tensile Strength, p.s.i. | Elongation in 2", Percent | Reduction of Area, Percent | V-Notch Charpy Impact Energy at Minus 60 F. Ft./Lb. |
|-------------|----------------------|--------------------------------------|--------------------------|---------------------------|----------------------------|-----------------------------------------------------|
| 1L725.....  | 3.36                 | 33,830                               | 129,350                  | 52.5                      | 44.2                       | 50—49                                               |
| 1L715.....  | 6.46                 | 44,780                               | 95,000                   | 62.0                      | 56.7                       | 166—159—155                                         |
| 1L547.....  | 8.17                 | 46,700                               | 98,300                   | 68.5                      | 75.3                       | 173—161                                             |
| 1L558.....  | 8.64                 | 60,950                               | 107,675                  | 65.0                      | 74.9                       | 236—236                                             |
| 1L673.....  | 9.42                 | 62,450                               | 102,900                  | 63.5                      | 73.0                       | 237—235                                             |
| 1L640.....  | 12.29                | 61,670                               | 119,500                  | 58.5                      | 66.0                       | 189—174                                             |
| 1L638.....  | 15.41                | 60,700                               | 110,750                  | 67.0                      | 71.1                       | 97                                                  |
| 1L724.....  | 15.69                | 59,850                               | 109,975                  | 52.0                      | 46.5                       | 96—89                                               |

GROUP Ia

|            |       |            |            |            |            |    |
|------------|-------|------------|------------|------------|------------|----|
| 1L890..... | 14.11 | Not Tested | Not Tested | Not Tested | Not Tested | 51 |
| 1L881..... | 14.29 | Not Tested | Not Tested | Not Tested | Not Tested | 72 |

GROUP II

|             |       |        |         |      |      |             |
|-------------|-------|--------|---------|------|------|-------------|
| 1L1003..... | 11.74 | 56,500 | 106,000 | 53.5 | 71.5 | 208—184     |
| 1L1002..... | 12.56 | 56,500 | 108,000 | 55.0 | 70.5 | 200—184     |
| 1L1005..... | 12.83 | 60,000 | 110,000 | 53.0 | 71.5 | 204—176     |
| 1L1009..... | 13.11 | 52,000 | 105,200 | 52.5 | 70.0 | 198—182     |
| 1L1004..... | 13.37 | 57,000 | 107,000 | 55.0 | 68.0 | 208—186     |
| 1L1006..... | 13.74 | 57,695 | 107,900 | 55.0 | 69.2 | 194—191     |
| 1L1092..... | 13.77 | 61,815 | 116,400 | 60.3 | 71.0 | 217—214     |
| 1L095.....  | 13.98 | 61,500 | 115,000 | 53.0 | 69.9 | 240—226—222 |
| 1L1090..... | 14.71 | 58,190 | 110,350 | 55.5 | 71.0 | 237—235—194 |
| 1L1091..... | 15.28 | 59,815 | 115,125 | 53.8 | 70.0 | 240—221—210 |

GROUP IIa

|             |       |        |         |      |      |             |
|-------------|-------|--------|---------|------|------|-------------|
| 1L1096..... | 6.98  | 55,570 | 110,950 | 56.0 | 70.1 | 233—225—214 |
| 1L1095..... | 9.88  | 55,840 | 110,460 | 53.0 | 70.6 | 240—240—240 |
| 1L1094..... | 12.93 | 56,220 | 108,330 | 54.0 | 72.3 | 236—224—220 |

Results of high temperature oxidation tests of the steels of Table I are given in the following Table III:

TABLE III.—RESULTS OF 78-HOUR OXIDATION TESTS AT 1500° F. IN THE ANNEALED CONDITION

| GROUP I     |                      |                          |                               |
|-------------|----------------------|--------------------------|-------------------------------|
| Heat Number | Total Cr+Al, Percent | Weight Gain, mg./sq. cm. | Appearance After Exposure     |
| 1L725       | 3.36                 | 72.2                     | Heavy layers of loose scale.  |
| 1L715       | 6.46                 | 33.5                     | Do.                           |
| 1L647       | 8.17                 | 1.1                      | Fine dust-like scale.         |
| 1L583       | 8.54                 | 8.1                      | Do.                           |
| 1L572       | 9.42                 | 1.2                      | Do.                           |
| 1L640       | 12.29                | 1.5                      | Do.                           |
| 1L638       | 15.41                | Not tested               | Bright, no evidence of scale. |
| 1L724       | 15.69                | 0.2                      |                               |

GROUP Ia

| Heat Number | Total Cr+Al, Percent | Weight Gain, mg./sq. cm. | Appearance            |
|-------------|----------------------|--------------------------|-----------------------|
| 1L830       | 14.11                | 0.8                      | Discolored.           |
| 1L831       | 14.29                | 6.1                      | Fine dust-like scale. |

GROUP II

| Heat Number | Total Cr+Al, Percent | Weight Gain, mg./sq. cm. | Appearance            |
|-------------|----------------------|--------------------------|-----------------------|
| 1L1003      | 11.74                | 1.6                      | Trace of loose scale. |
| 1L1032      | 12.56                | Not tested               | Do.                   |
| 1L1005      | 12.83                | 0.9                      | Do.                   |
| 1L1009      | 13.11                | 0.8                      | Do.                   |
| 1L1004      | 13.37                | 0.6                      | Do.                   |
| 1L1003      | 13.75                | 0.7                      | Do.                   |
| 1L1002      | 13.77                | 2.9                      | Fine loose scale.     |
| 1L695       | 13.98                | 3.8                      | Do.                   |
| 1L1030      | 14.71                | 4.7                      | Do.                   |
| 1L1031      | 15.28                | 1.9                      | Do.                   |

Cold formability results as determined by 180 degree bend tests in the annealed and sensitized condition for the steels of Table I are given in the following Table IV:

TABLE IV.—RESULTS OF 180 DEGREE BEND TESTS IN THE ANNEALED AND SENSITIZED CONDITION

| GROUP I     |                      |                                          |                                                                     |
|-------------|----------------------|------------------------------------------|---------------------------------------------------------------------|
| Heat Number | Total Cr+Al, Percent | As Annealed (2/3 Hr. at 2,000° F., W.Q.) | Annealed and Sensitized (2,000° F., W.Q.+2 Hrs. at 1,250° F., A.C.) |
| 1L725       | 3.36                 | No evidence of cracking.                 | No evidence of cracking.                                            |
| 1L715       | 6.46                 | do.                                      | Do.                                                                 |
| 1L647       | 8.17                 | do.                                      | Do.                                                                 |
| 1L583       | 8.54                 | do.                                      | Do.                                                                 |
| 1L572       | 9.42                 | do.                                      | Do.                                                                 |
| 1L640       | 12.29                | do.                                      | Do.                                                                 |
| 1L638       | 15.41                | do.                                      | Do.                                                                 |
| 1L724       | 15.69                | do.                                      | Brittle break at start of bending.                                  |

GROUP Ia

| Heat Number | Total Cr+Al, Percent | As Annealed (2/3 Hr. at 2,000° F., W.Q.) | Annealed and Sensitized (2,000° F., W.Q.+2 Hrs. at 1,250° F., A.C.) |
|-------------|----------------------|------------------------------------------|---------------------------------------------------------------------|
| 1L830       | 14.11                | No evidence of cracking.                 | No evidence of cracking.                                            |
| 1L831       | 14.29                | do.                                      | Do.                                                                 |

GROUP II

| Heat Number | Total Cr+Al, Percent | As Annealed (2/3 Hr. at 2,000° F., W.Q.) | Annealed and Sensitized (2,000° F., W.Q.+2 Hrs. at 1,250° F., A.C.) |
|-------------|----------------------|------------------------------------------|---------------------------------------------------------------------|
| 1L1003      | 11.74                | No evidence of cracking.                 | No evidence of cracking.                                            |
| 1L1002      | 12.56                | do.                                      | Do.                                                                 |
| 1L1005      | 12.83                | do.                                      | Do.                                                                 |
| 1L1009      | 13.11                | do.                                      | Do.                                                                 |
| 1L1004      | 13.37                | do.                                      | Do.                                                                 |
| 1L1006      | 13.75                | do.                                      | Do.                                                                 |
| 1L1002      | 13.77                | do.                                      | Do.                                                                 |
| 1L695       | 13.98                | do.                                      | Do.                                                                 |
| 1L1030      | 14.71                | do.                                      | Do.                                                                 |
| 1L1031      | 15.28                | do.                                      | Do.                                                                 |

GROUP IIa

| Heat Number | Total Cr+Al, Percent | As Annealed (2/3 Hr. at 2,000° F., W.Q.) | Annealed and Sensitized (2,000° F., W.Q.+2 Hrs. at 1,250° F., A.C.) |
|-------------|----------------------|------------------------------------------|---------------------------------------------------------------------|
| 1L1036      | 6.98                 | No evidence of cracking.                 | No evidence of cracking.                                            |
| 1L1035      | 9.88                 | do.                                      | Do.                                                                 |
| 1L1034      | 12.93                | do.                                      | Do.                                                                 |

6  
Typical properties of Steels A, B and C in the annealed condition are given in the following Table V:

TABLE V  
PROPERTIES—ANNEALED

| Steels                                           | A       | B       | C       |
|--------------------------------------------------|---------|---------|---------|
| Yield Strength, 0.2% Offset                      | 50,000  | 60,000  | 60,000  |
| Tensile Strength                                 | 105,000 | 110,000 | 110,000 |
| Elongation in 2 Inches, percent                  | 65.0    | 60.0    | 50.0    |
| Reduction of Area, percent                       | 70.0    | 65.0    | 45.0    |
| V-Notch Charpy Impact Energy at -60° F., ft./lb. | 235     | 170     | 90.0    |

  

| OXIDATION RESISTANCE                                     |     |     |     |
|----------------------------------------------------------|-----|-----|-----|
| 78-Hours at 1,500 F., Weight Gained mg./cm. <sup>2</sup> | 2.0 | 1.0 | 0.2 |

Steel A is characterized by a completely austenitic structure in the solution annealed condition. A unique feature of this composition is that it remains relatively free of carbide precipitation after forging and after annealing and sensitizing in the range of 1100 to 1400 F. It is further characterized by high tensile and yield strengths, high tensile ductility, excellent impact ductility, and fair oxidation resistance. This steel can be hot and cold formed and provides the foregoing combinations of properties economically. A typical use is for automobile mufflers and for other applications requiring these improved properties at minimum cost.

Steel B is characterized by a completely austenitic structure in the annealed condition. It is further characterized by high tensile and yield strengths, high tensile ductility, high impact ductility, good oxidation resistance at elevated temperatures, and atmospheric corrosion resistance. This steel can be hot and cold formed and provides the properties of Steel A along with improved atmospheric corrosion resistance and improved elevated-temperature oxidation resistance.

Steel C is characterized by an austenitic structure in the solution annealed condition. This steel provides somewhat better atmospheric corrosion and oxidation resistance than Steels A and B with some sacrifice of tensile and impact ductility and hot workability. Thus it is suitable for such uses as automobile trim since it has good corrosion resistance and good cold workability.

Contradistinguished from the foregoing is the following steel which is a typical steel of the prior art.

| Heat No.    | Chemical Composition, Weight Percent |       |      |       |      |               |
|-------------|--------------------------------------|-------|------|-------|------|---------------|
|             | C                                    | Mn    | Si   | Cr    | Al   | Percent Cr+Al |
| 1L1125..... | 0.99                                 | 10.90 | 0.61 | 22.71 | 2.68 | 25.39         |

The annealed and impact properties of this Steel 1L1125 are given in the following Table VI:

TABLE VI.—ANNEALED TENSILE AND IMPACT PROPERTIES\*

| Heat Number | Total Cr+Al, Percent | Yield Strength (0.2% Offset), p.s.i. | Tensile Strength, p.s.i. | Elongation in 2", Percent | Reduction of Area, Percent | V-Notch Charpy Impact Energy at Minus 60° F., Ft./Lb. |
|-------------|----------------------|--------------------------------------|--------------------------|---------------------------|----------------------------|-------------------------------------------------------|
| 1L1125..... | 25.39                | 76,500                               | 84,800                   | 3.0                       | 6.00                       | 4                                                     |

\*Annealed at 2,000° F. and water quenched.

Oxidation and cold formability tests on this steel are given in the following Tables VII and VIII:

TABLE VII.—RESULTS OF 78-HOUR OXIDATION TEST AT 1500° F. IN THE ANNEALED CONDITION

| Heat No.    | Total Percent Cr+Percent Al | Weight Gain, mg./cm. <sup>2</sup> |
|-------------|-----------------------------|-----------------------------------|
| 1L1125..... | 25.39                       | 1.0                               |

TABLE VIII.—RESULTS OF 180 DEGREE BEND TEST

| Heat Number | Total Cr+Al, percent | As Annealed 1/2 Hr. at 2000° F., W.Q. | Annealed and Sensitized (2000° F., W.Q.+2 Hrs. at 1250° F., A.C.) |
|-------------|----------------------|---------------------------------------|-------------------------------------------------------------------|
| 1L1125..... | 25.39                | Brittle break at start of bending.    | Brittle break at start of bending.                                |

The poor tensile and impact ductility of such prior steel of Heat No. 1L1125 is clearly shown by the foregoing data.

From the foregoing it is apparent that the steels of this invention are characterized by an austenitic structure in the solution annealed condition, high tensile and yield strengths, good tensile and impact ductility, good atmospheric corrosion resistance and elevated-temperature oxi-

dation resistance along with good hot and cold formability properties.

While we have shown and described several specific embodiments of our invention, it will be understood that these embodiments are merely for the purpose of illustration and description and that various other forms may be devised within the scope of our invention, as defined in the appended claims.

We claim:

1. An aluminum-bearing, non-age-hardening austenitic steel characterized by high temperature oxidation resistance, good cold formability and low temperature impact properties, said steel consisting essentially of

|               | Percent      |
|---------------|--------------|
| Carbon        | .25 to 1.0   |
| Manganese     | 14.0 to 35.0 |
| Silicon       | .25 to 1.0   |
| Chromium      | 4.5 to 8.75  |
| Aluminum      | 3.5 to 8.75  |
| Balance iron. |              |

wherein the carbon, manganese, chromium and aluminum are balanced to provide an austenitic structure and where-

in the chromium and aluminum are balanced within the following limits

Percent chromium=percent aluminum-1.5

to

Percent chromium=percent aluminum+1.5

with the total of percent chromium plus percent aluminum being less than 17.

2. An aluminum-bearing, non-age-hardening austenitic steel characterized by high temperature oxidation resistance, good cold formability and low temperature impact properties, said steel consisting essentially of

|                   | Percent      |
|-------------------|--------------|
| Carbon            | .40 to .90   |
| Manganese         | 14.0 to 18.0 |
| Silicon           | .35 to .75   |
| Chromium          | 4.5 to 8.50  |
| Aluminum and iron | 3.75 to 8.50 |

wherein the carbon, manganese, chromium and aluminum are balanced to provide an austenitic structure and where-in the chromium and aluminum are balanced within the following limits

Percent chromium=percent aluminum-1.5

to

Percent chromium=percent aluminum+1.5

with the total of percent chromium plus percent aluminum being between 9 and 16.

3. An aluminum-bearing, non-age-hardening austenitic steel characterized by good corrosion resistance, high tem-

perature oxidation resistance, low temperature impact properties, high tensile properties and good cold formability, said steel consisting essentially of

|           | Percent    |
|-----------|------------|
| Carbon    | About 0.50 |
| Manganese | About 15.0 |
| Silicon   | About 0.50 |
| Chromium  | About 5.0  |
| Aluminum  | About 4.0  |

with the balance iron.

4. An aluminum-bearing, non-age-hardening austenitic steel characterized by good corrosion resistance, high temperature oxidation resistance, low temperature impact properties, high tensile properties and good cold formability, said steel consisting essentially of

|           | Percent    |
|-----------|------------|
| Carbon    | About 0.80 |
| Manganese | About 16.0 |
| Silicon   | About 0.50 |

10

|          | Percent    |
|----------|------------|
| Chromium | About 7.00 |
| Aluminum | About 6.00 |

with the balance iron.

5. An aluminum-bearing, non-age-hardening austenitic steel characterized by good corrosion resistance, high temperature oxidation resistance, low temperature impact properties, high tensile properties and good cold formability, said steel consisting essentially of

|           | Percent     |
|-----------|-------------|
| Carbon    | About 0.90  |
| Manganese | About 17.00 |
| Silicon   | About 0.50  |
| Chromium  | About 8.00  |
| Aluminum  | About 7.00  |

with the balance iron.

No references cited.

DAVID L. RECK, Primary Examiner.

UNITED STATES PATENT OFFICE  
CERTIFICATE OF CORRECTION

Patent No. 3,201,230

August 17, 1965

Joseph R. Mitchell et al.

It is hereby certified that error appears in the above numbered patent requiring correction and that the said Letters Patent should read as corrected below.

Column 1, line 14, for "fuel" read -- steel --; column 2, TABLE I, second column, line 6 thereof, for "0.85" read -- 0.86 --; column 3, TABLE I-Continued, GROUP Ia, fourth column, line 1 thereof, for "0.103" read -- 0.013 --; same table, tenth column, line 2 thereof, for "0.96" read -- 1.96 --; same table, GROUP II, fifth column, line 1 thereof, for "0.104" read -- 0.014 --; same table, eighth column, line 4 thereof, for "5.80" read -- 5.90 --; same column 3, line 31, after "percent", first occurrence, insert -- chromium --; column 5, TABLE III, GROUP I, fourth column, line 7 thereof, strike out "Bright, no evidence of scale.", and insert the same in the same column, line 8, and opposite Heat Number "11L724"; same table, GROUP II, fourth column, line 2 thereof, strike out "Do.".

Signed and sealed this 5th day of April 1966.

(SEAL)

Attest:

ERNEST W. SWIDER  
Attesting Officer

EDWARD J. BRENNER  
Commissioner of Patents